# EUROPEAN PATENT SPECIFICATION

(11) **EP 0 084 910 B1**
(45) Date of publication and mention of the grant of the patent: **22.02.1989**
(21) Application number: 83200077.2
(22) Date of filing: 18.01.1983
(51) Int. Cl.: C10M 123/02, C10M 129/54, C10M 135/10, C10M 143/00, C10M 149/02, C10M 155/04, C10N 30/00

(54) **High dropping-point lithium-complex grease having improved anti-noise properties**
Lärmverhinderde Eigenschaften aufweisendes Lithium-Komplex-Fett mit hohem Tropfpunkt
Graisse à haut point de goutte avec des propriétés anti-bruit améliorées contenant un complexe de lithium

(30) Priority: 21.01.1982 JP 6757/82; 21.01.1982 JP 6758/82
(43) Date of publication of application: 03.08.1983
(73) Proprietor: SHELL INTERNATIONALE RESEARCH MAATSCHAPPIJ B.V., 2596 HR Den Haag (NL)
(72) Inventor: Tanaka, Norimitsu, Takatsu-ku Kawasaki City (JP); Tajiri, Hiroshi, Sagamihara City Kanagawa Pref. (JP); Okamoto, Toshiko, Takatsu-ku Kawasaki City (JP)
(74) Representative: Aalbers, Onno

(56) References cited:
- US-A- 3 929 650
- US-A- 3 929 651
- US-A- 4 100 080
- US-A- 4 156 655

## Description

The present invention relates to a high-quality lithium-complex grease composition having improved anti-noise properties, a high dropping point, a long lubrication life and an excellent oxidation stability also at high temperatures.

High dropping-point lithium-soap greases are generally referred to as lithium-complex greases, and several of them are proposed so far (see e.g. US patent specifications 2,940,930, 3,223,624, 3,758,407 and 3,929,651). However, these lithium-complex greases were inferior in their anti-noise properties because of the low dispersancy in the base oils of the metal salts used for the formation of complexes with lithium soaps.

The purpose of the present invention is to provide a lithium-complex grease composition having a long lubrication life, markedly improved anti-noise properties, a high dropping point, and an excellent oxidation stability also at high temperatures, by uniformly admixing and dispersing in a base lubricating oil a gelling agent (a), a complexing metal salt (b) and a dispersing component (c). From US-A-3,929,650 grease compositions are known comprising a thickener system of lithium hydroxy stearate and lithium borate. The composition may further contain an alkaline earth metal sulphonate and optionally a succinimide derived from alkenyl succinic acid or anhydride and alkylene polyamines.

GS-A-4,165,655 discloses a grease composition containing a lithium salt of a C₁₂-₂₄ hydroxy fatty acid, mono lithium borate and a metal naphthenate and a quaternary ammonium salt.

Grease compositions containing the lithium salt of a C₁₂-₂₄ hydroxy fatty acid and the dilithium salt of azelaic, sebacic, or adipic acid and lithium salicylate, are known from US-A-3,929,651. These compositions may further comprise a naphthalene sulphonate and/or an alkylmethacrylate polymer.

The greases according to the present invention have improved anti-noise characteristics in comparison with these known compositions.

This invention therefore relates to a high dropping-point lithium-complex grease composition having improved anti-noise properties, comprising a lubricating oil and the following components:
(a) at least one lithium soap selected from the group consisting of the lithium salts of C₁₀ to C₃₄ fatty acids and C₁₂ to C₂₄ hydroxy fatty acids,
(b) at least one lithium salt selected from the group consisting of the dilithium salts of adipic acid, sebacic acid or azelaic acid and lithium salicylate, and
(c) at least one dispersing component, characterized in that component (c) is selected from the group consisting of hydrogenated styrene-butadiene copolymers, hydrogenated styrene-isoprene copolymers and ethylene-propylene copolymers, if component (b) is a dilithium salt of adipic, sebacic and/or azelaic acid; and component (c) is selected from the group consisting of a succinimide-type dispersant of formulae wherein A¹ denotes a C₃₀ to C₂₀₀ polyisobutyl radical, p means an integer from 2 to 8 and q represents an integer from 1 to 8, and calcium sulphonate, calcium salicylate and magnesium salicylate of formulae wherein A² and A^{2'} are respectively a hydrogen atom or a Cₐ to C₃₀ alkyl radical; Ar means a benzene or naphthalene ring, A⁵ means a C₈ to C₂₂ alkyl radical and M¹ denotes Ca or Mg, if component (b) is lithium salicylate.

### Lubricating oil

Any conventional lubricating oil can be used. While a typical one is a mineral oil, use can also be made, singly or in combination with the mineral oil, of a synthetic oil including ester oils, such as a diester oil, e.g. dioctyl azelate, and a tetra-ester oil, e.g. the pentaerythritol ester of an aliphatic monocarboxylic acid, or poly-alpha-olefin oligomers, such as octene-1/-decene-1 copolymers, having viscosity of 41.0 cSt at 37.7°C, a viscosity index (V.I.) of 130 and a flash point of 223°C.

The lubricating oil may have a viscosity ranging from about 2 to 500 cSt, preferably from 20 to 200 cSt, at 40°C.

### Component (a)

The C_{IO} to C₃₄ fatty acids include the saturated or unsaturated higher aliphatic monocarboxylic acids, especially those acids containing 16 to 22 carbon atoms, such as stearic acid and oleic acid.

The C₁₂ to C₂₄ hydroxy fatty acids include saturated or unsaturated monocarboxylic fatty acids containing a hydroxyl radical, especially those acids containing 18 carbon atoms and a hydroxyl radical in the 9-, 10-, or 12- position, such as 12-hydroxy stearic acid and ricinolic acid.

The lithium salts of the above fatty acids and hydroxy fatty acids can be singly used or combinedly with one or more of others. In addition, when said lithium salts are prepared, said carboxylic acids can be reacted with lithium hydroxide not only in the form of free acids but also as glycerides.

### Component (c)

This component is used for the acceleration of the fine dispersion of the components (a) and (b) in the base oil, and the compounds mentioned can be employed singly or combinedly with one or more of other ones.

Conventional VI-improvers can be used, such as:
1. hydrogenated styrene-butadiene copolymers, especially those of the mean molecular weights ranging from 20,000 to 250,000 and styrene contents ranging from 25 to 70 weight %;
2. hydrogenated styrene-isoprene copolymers, especially those of the mean molecular weights ranging from 20,000 to 250,000 and styrene contents ranging from 20 to 65 weight%;
3. ethylene-propylene copolymers, especially those of the mean molecular weights ranging from 20,000 to 250,000 and ethylene contents ranging from 10 to 30 weight%.

Suitable succinimide type dispersants are synthesized by reaction of polyamines with the polybutenyl succinic anhydrides obtained by the reaction of polybutenes and maleic anhydride.

The suitable metal salts used as component (c) may be neutral, basic or super-basic. Combinations of the metal salts may also be suitable.

### Preparation of grease composition

The grease composition according to the present invention can be prepared by uniformly admixing and finely dispersing the three components (a), (b) and (c) in the base oil mentioned above. While the amounts of these three components compounded in the base oil above are not necessarily critical but can be variable for individual components, it is generally advantageous to use them in the following proportions per 100 weight parts (pbw) of the base oil;
Component (a): 2 to 40 weight parts, preferably 5 to 30 weight parts
Component (b): 0.05 to 20 weight parts, preferably 0.5 to 10 weight parts
Component (c): 0.01 to 10 weight parts, preferably 0.1 to 5 weight parts.

Also, it is particularly preferable to use the components (a) and (b) in the following mol ratio within the above ranges of the proportions;

Component (a)/Component (b) mol ratio=0.5 to 10, especially 1 to 5.

In the grease composition according to the present invention, use can be made, in addition to the three components (a), (b) and (c) above, of other ordinary lubricant-additives, such as neutral or basic metallic detergents, such as basic Ca salicylate, or ashless dispersants, rust inhibitors (e.g., paraffin oxide, amino imidazoline or barium dinonlynaphthalene-sulphonate), oxidation inhibitors (e.g. 2,6-ditertiary butyl-4-methylphenol, N-phenyl- -naphthylamine or diphenylamine octylate) and extreme-pressure additives (e.g. zinc naphthenate, or other zinc compounds such as zinc dithiophosphates or zinc-oxide, lead naphthenate, sulphurized oils and fats, or tricresyl phosphate), in the proportions ordinarily employed.

The grease composition of the present invention can e.g. be prepared in the following manner.

A component (c) is first admixed and dissolved in a base oil, and the fatty acid or hydroxy fatty acid for the preparation of the lithium soap, as a component (a), is admixed and dissolved in the mixture thus obtained, at 70 to 80°C. Then, the lithium hydroxide roughly in an equivalent amount to the fatty acid or hydroxy fatty acid above is admixed in the resulting mixture at 80 to 90°C to form a soap, and the mixture is further heated to 140 to 150°C under pressure for dehydration. After the dicarboxylic acid for the formation of a component (b) is admixed in the dehydrated mixture, the resulting mixture is cooled to 80 to 100°C and further admixed with the lithium hydroxide roughly in an equivalent amount to said dicarboxylic acid and the final mixture is again dehydrated by heating to 140 to 150°C under pressure. The last dehydrated mixture is further heated to 195 to 215°C, then cooled to 175 to 193°C, maintained at this temperature for about 10 to 40 min. and finally cooled to the room temperature.

The lithium complex grease composition according to the present invention and thus prepared has a very high dropping point, satisfactory anti-noise properties and very long lubricating life and exhibits exceedingly high performance as a lubricating grease. Therefore, the present grease composition can be suitably used, for example, for the lubrication of the bearings fitted in electric motors as well as of the wheel bearings in automotive bearing/axie integrated structures. Furthermore, these greases make little noise even if used in the bearings of air-conditioners and others, giving no environmental injury.

The invention is illustrated in Examples 1, 3, 5-8, 14 and 16-22 below. Examples 2, 4, 9-13, 15, 23 and 24 are included for comparative purposes.

### Example 1

2,233.5g of a refined mineral oil (paraffinic, VI:102, pour pt. -15°C, viscosity: 44.9 cSt at 37.8°C and 6.4 cSt at 98.9°C), 300g of the 10% solution of a hydrogenated styrene-butadiene copolymer (mesh mol. wt.: about 130,000, styrene content: 59 weight %) in the mineral oil above and 270g of 12-hydroxy stearic acid were charged into a 8 litre autoclave, and the contents were heated to 80°C under stirring in 30 to 40 min to completely dissolve the 12-hydroxy stearic acid.

Then, 300g of a hot aqueous solution (95°C) containing 38.5g of lithium hydroxide were admixed in the autoclave, the contents were stirred for about 10 min under stirring and normal pressure at about 90°C and, then, slowly heated under pressure to about 145°C. At this temperature, the contents of the autoclave were further stirred for about 15 min under pressure (about 2.5 to 2.8kg/cm²) and, subsequently, the pressure was released with the moisture being removed.

After dehydration, the contents were admixed with 67.8g of azelaic acid, the mixture was slowly cooled to about 90°C under stirring, and 250g of a hot aqueous solution (95°C) containing 30.2g of lithium hydroxide were admixed in the mixture. The resulting mixture was slowly heated to 145 to 155°C under stirring and pressure in 1 to 1.5 hrs, and, at this temperature, the autoclave was released of the pressure and removed of the moisture.

After the dehydration, the contents of the autoclave were again heated to 195 to 215°C and, then, left cooling under stirring to 188 to 192°C. The contents were kept at this temperature for 20 to 30 min, then left cooling to about 160°C. At this temperature 60g of the oxidation inhibitor, diphenylamine octylate, were admixed in the contents, the mixture was cooled to about 80 to 85°C under stirring in 30 to 60 min and treated in a homogenizer at this temperature.

The properties of the grease composition thus obtained were as shown below:

### Comparison Example 2

A grease composition was prepared in a similar manner to that in Example 1 except that 2,533.5g of the refined mineral oil were used without employing the hydrogenated styrene-butadiene copolymer mentioned in Example 1. The properties of the product were as follows:

### Examples 3 to 8

Grease compositions were prepared by employing the various components shown in Table 1 below in a similar manner to that in Example 1, and the properties of these compositions are collectively tabularized in Table 1.

### Example 9

Grease composition 9 was prepared by treating the various components shown in following Table 2 in similar manners to that in Example 1. The properties of this composition are shown in Table 2.

39 weight parts of the compound above dissolved in 100 weight parts of the refined mineral oil.

### Examples 10 to 13

Grease compositions were prepared by treating the various components shown in following Table 3 in similar manners to that in Example 1. The properties of these compositions are collectively tabularized in Table 3.

### Example 14

2,521.2g of a refined mineral oil (paraffinic, VI; 102, pour point: -15°C, kin, viscosity: 44.9 cSt at 37.8°C, 6.4 cSt at 98.9°C), 30g of a succinimide (A) (ref. Note 1) and 270g of 12-hydroxy stearic acid were introduced into a liter autoclave and the contents were heated to 80°C under stirring in 30 to 40 min to completely dissolve the hydroxystearic acid. (Note 1: Succinimide (A) A': C₅₂ to C₇₆ polyisobutenyl radical, mean molecular weight: 2,302 (as containing boron), 110wt. parts of the compound above dissolved in 100wt. parts of the base oil).

Subsequently, 300g of a hot aqueous solution (95°C) containing 38.5g of lithium hydroxide were admixed in the autoclave contents, which were then kept at 90°C under stirring for 5 to 15 min. After the contents were cooled to 75°C, 300g of a hot aqueous solution (93°C) containing 49.8g of salicylic acid were admixed in the contents and dissolved by stirring for 10 to 15 min. Then, 250g of a hot aqueous solution (95°C) containing 31.0 of lithium hydroxide were admixed in the resulting mixture, which was then gradually heated under stirring and pressure. When this mixture arrived at 145 to 150°C after 1 to 1.5 hrs, the autoclave was released of the pressure and the contents of were dehydrated at this temperature in 15 to 25 min. After the dehydration, the contents of the autoclave were further heated to 195 to 205°C, then cooled to 188 to 192°C under stirring and, after being kept at this temperature for 20 to 30 min, further cooled to about 160°C. At this temperature, 60g of an oxidation inhibitor were admixed in the contents, the mixture thus obtained was cooled by stirring to about 80 to 85°C in 30 to 60 min and then treated in a homogenizer at this temperature.

The properties of the grease composition thus prepared were as follows:

### Example 15

A grease composition was prepared in a similar manner to that in Example 1 except that 2,531.2g of the refined mineral oil were employed without the succinimide (A) being admixed, the properties of the resulting composition were as follows;

### Examples 16 to 24

Seven grease compositions were prepared by treating the various components shown in Table 4 below in similar ways to that in Example 26 and the properties thereof are collectively tabularized in Table 4. Also, the properties of a market grease comprising the lithium soap of 12-hydroxystearic acid are shown as Example 23 in the table as well. In addition, in Example 24 in the Table a grease is prepared in a similar manner to that in Example 14 but by employing an increased amount of the refined mineral oil without the components (b) and (c) being admixed.

A¹: C₅₂ to C₇₆ polyisobutenyl radical.
Mean molecular weight: 2,170.

110 weight parts of the above compound dissolved in 100 weight parts of a refined mineral oil. (2)
A¹: C₅₂ to C₇₆, polyisobutenyl radical.
Mean molecular weight: 1,172.

160 weight parts of the above compound dissolved in 100 weight parts of a refined mineral oil. (3)
A¹: C₅₂ to C₇₆ polyisobutenyl radical.
Mean molecular weight: 1,304.

140 weight parts of the compound above dissolved in 100 weight parts of a refined mineral oil. (4) Calcium dinonylnaphthalene-sulphonate

39 weight parts of the compound above dissolved in 100 weight parts of a refined mineral oil. (5) Magnesium alkyl-salicylate
R: C₁₀ to C₁₆ alkyl radical.

30 weight parts of the compound above dissolved in 100 weight parts of a refined mineral oil. (6) Calcium alkyl-salicylate
R: C₁₀ to C₁₆ alkyl radical.

30 weight parts of the compound dissolved in 100 weight parts of a refined mineral oil. (7) The same as that used in Example 26. (8) The same as that used in Example 26.

Examples 1,3,5―8, 14, 16―22 are according to the present invention; Examples 2, 4, 9―13, 15, 23 and 24 have been included for comparison.

## Claims

1. High dropping-point lithium-complex grease composition having improved anti-noise properties, comprising a lubricating oil and the following components:
(a) at least one lithium soap selected from the group consisting of the lithium salts of C_{'o} to C₃₄ fatty acids and C₁₂ to C₂₄ hydroxy fatty acids,
(b) at least one lithium salt selected from the group consisting of the dilithium salt of adipic acid, sebacic acid or azelaic acid and lithium salicylate, and
(c) at least one dispersing component, characterized in that component (c) is selected from the group consisting of hydrogenated styrene-butadiene copolymers, hydrogenated styrene-isoprene copolymers and ethylene-propylene copolymers, if component (b) is a dilithium salt of adipic, sebacic and/or azelaic acid; and component (c) is selected from the group consisting of a succinimide-type dispersant of formulae wherein A' denotes a C₃₀ to C₂₀₀ polyisobutenyl radical, p means an integer from 2 to 8 and q represents an integer from 1 to 8, and calcium sulphonate, calcium salicylate and magnesium salicylate of formulae wherein A² and A^{2'} are respectively a hydrogen atom or a C₈ to C₃₀ alkyl radical, Ar means a benzene or naphthalene ring, A⁵ means a C₈ to C₂₂ alkly radical and M¹ denotes Ca or Mg, if component (b) is lithium salicylate.

## Patentansprüche

1. Lithium-Komplex-Schmiermittelzusammensetzung mit hohem Tropfpunkt mit verbesserten Lärmdämpfungseigenschaften, enthaltend ein Schmieröl und die folgenden Komponenten:
(a) mindestens eine Lithiumseife ausgewählt aus der Gruppe bestehend aus den Lithiumsalzen von C₁₀- bis C₃₄- Fettsäuren und C₁₂- bis C₂₄-Hydroxyfettsäuren,
(b) mindestens ein Lithiumsalz, ausgewählt aus der Gruppe bestehend aus dem Dilithiumsalz der Adipinsäure, Sebacinsäure oder Azelainsäure und Lithiumsalicylat, und
(c) mindestens eine dispergierende Komponente, dadurch gekennzeichnet, daß die Komponente (c) ausgewählt ist aus der Gruppe bestehend aus hydrierten Styrol-Butadien-Mischpolymerisaten, hydrierten Styrol-Isopren-Mischpolymerisaten und Äthylen-Propylen-Mischpolymerisaten, wenn die Komponente (b) ein Dilithiumsalz der Adipin-Sebacin- und/oder Azelainsäure ist; und das die Komponente (c) ausgewählt ist aus der Gruppe bestehend aus einem dispergierenden Mittel vom Succinimid-Typ der Formeln: in welchem A' einen C₃₀―C₂₀₀-Polyisobutenylrest darstellt, p eine ganze Zahl von 2 bis 8 bedeutet und q eine ganze Zahl von 1 bis 8 ist, und Calziumsulfonaten, Calciumsalicylaten und Magnesiumsalicylaten der Formeln in welchem A² und A^{2'} jeweils ein Wasserstoffatom oder ein C₈―C₃₀-Alkylrest sind, Ar ein Benzolring oder Naphthalinring ist, A⁵ eine C₈―C₂₂-Alkylrest ist und M' Ca oder Mg bedeutet, wenn die Komponente (b) Lithiumsalicylat ist.

## Revendications

1. Composition de graisse à haut point de goutte avec des propriétés antibruits améliorées, contenant un complexe de lithium, comprenant une huile lubrifiante et les composants suivants:
(a) au moins un savon de lithium choisi dans le groupe constitué par les sels de lithium des acides gras en C₁₀―C₃₄ et des hydroxyacides gras en C₁₂―C₂₄,
(b) au moins un sel de lithium choisi dans le groupe constitué par les sels de dilithium de l'acide adipique, de l'acide sébacique ou de l'acide azélaïque et le salicylate de lithium, et
(c) au moins un composant dispersant, caractérisée en ce que le composant (c) est choisi dans le groupe constitué par les copolymères hydrogénés de styrène-butadiène, les copolymères hydrogénés de styrène-isoprène et les copolymères d'éthylène-propylène lorsque le composant (b) est un sel de dilithium d'acide adipique, sébacique et/ou azélaïque; et le composant (c) est choisi dans le groupe constitué par un dispersant de type succinimide répondant aux formules dans lesquelles A¹ représente un radical polyisobutényle en C₃₀ à C₂₀₀, p est un entier de 2 à 8 et q représente un entier de 1 à 8, et le sulfonate de calcium, salicylate de calcium et salicylate de magnésium de formules dans lesquelles A² et A^{2'} sont respectivement un atome d'hydrogène ou un radical alkyle en C₈ à C₃₀; Ar est un cycle benzène ou naphtalène, A⁵ est un radical alkyle en C⁸ à C₂₂ et M¹ est Ca ou Mg, lorsque le composant (b) est le salicylate de lithium.
